

Aug. 9, 1966

A. LICHTE

3,265,525

METHOD AND APPARATUS FOR CONTINUOUS COATING  
OF ENDLESS METAL BANDS WITH  
SYNTHETIC RESINS

Filed April 1, 1963

2 Sheets-Sheet 1

Fig. 1



Aug. 9, 1966

A. LICHTE

3,265,525

METHOD AND APPARATUS FOR CONTINUOUS COATING  
OF ENDLESS METAL BANDS WITH  
SYNTHETIC RESINS

Filed April 1, 1963

2 Sheets-Sheet 2

Fig. 2



Fig. 4



Fig. 3



## 1

3,265,525

**METHOD AND APPARATUS FOR CONTINUOUS COATING OF ENDLESS METAL BANDS WITH SYNTHETIC RESINS**

Albert Lichte, Wuppertal-Elberfeld, Germany, assignor to Schloemann Aktiengesellschaft, Dusseldorf, Germany, a German company

Filed Apr. 1, 1963, Ser. No. 269,394

Claims priority, application Germany, Apr. 4, 1962, Sch 31,252

4 Claims. (Cl. 117—49)

This invention relates to a method of and apparatus for the bubble-free coating of thin layers of synthetic material, in a liquid or pasty condition, in a continuous operation, upon continuously occurring endless metal bands, and for the rapid hardening of the layer of synthetic material so applied.

The synthetic coating material may consist of mixed PVC polymerizes, acrylic resins, alkyds, or certain proprietary preparations of the kind commonly known as plastic lacquers.

The object of the invention is to carry out the coating and hardening in a small space, with simple apparatus and small operative expenditure, in as short a time as possible. In particular, the drying or gelatinising and hardening times are to be short, and a rapid change-over to different materials and orders of magnitude, with dust-free working, is to be rendered possible.

The invention consists in applying the synthetic material, which has been brought into a pasty to liquid condition by means of a solvent of the ketone group for example, to the band to be coated, in a vacuum, and effecting the hardening or polymerisation of the applied layer in a vacuum, or at least in a treatment chamber at a lowered pressure. (When reference is hereinafter made to vacuum, what is meant is a lowered pressure which is less than atmospheric pressure). Owing to the fact that in a vacuum the fractional distillation of the solvent can be reduced by lowering the boiling points of the participating solvents, the gelatinising, drying or polymerising process, which is controlled by the solvents, admits of being considerably shortened. The usual solvents, for instance methyl ethyl ketone, evaporate in a normal atmosphere at about 80° C. By adopting a slightly lowered pressure, between 100 and 40 Torr (millimetres of mercury) for example, the boiling point can be shifted to room temperature or lower. This has the advantage that following the vaporisation of the solvents a cooling of the coated band in the conventional sense is no longer required. The entire drying tract for the hardening of the coating is thereby considerably shortened, so that a considerable increase in the speed of passage of the band is possible. Besides the advantages of a greater coating output, the coating materials applied in a vacuum are free from bubbles and free from dust. Additional advantages are yielded by the vacuum treatment, in that the solvent vapours arising from the vaporisation of the solvents can be condensed by appropriate cooling devices and collected. The consumption of solvents can thereby be considerably reduced. Furthermore, in the coating of light metals, aluminium bands for example, there is an advantage, in that no alteration in the technological properties of the aluminium band is brought about, because the drying in a vacuum is effected below the recrystallisation temperature.

Finally, as compared with conventional coating installations, a substantially smaller consumption of energy is also an advantage, for only the heat of vaporisation eliminated in the evaporation of the solvents need be resupplied. This supply of heat, which is in any case necessary for the maintenance of the vaporisation temperature, is however comparatively small.

## 2

The apparatus for carrying out the process according to the invention, which comprises a vacuum chamber serving for the vacuum treatment, closed in an airtight manner, at both the band-admission and the band-exit ends, in a known manner by vessels containing liquid, is characterised by the feature that at the same level as the sealing-liquid containers, and between these, treatment vessels are provided, and that the sealing-liquid vessels are in each case connected by way of one connecting tube, but the treatment vessels in each case by way of two connecting tubes, with a vacuum tank arranged above at a higher level, in such a way that the band to be coated can be carried through the apparatus in a number of vertical loops, the reversing rollers that carry the band, and also the actual coating appliances, being arranged partly in the sealing and treatment vessels and partly in the vacuum tank.

The installation costs of this apparatus, as compared with conventional plants, are extremely low. The vacuum chamber, having regard to the purpose for which it is employed, is by this arrangement kept very small, and owing to the vertical tube connection of the liquid vessels with the upper vacuum tank, the provision of as high a vacuum as may be desired is possible, since the column of liquid sucked up by the vacuum in these connecting tubes can be raised as far as may be wished. Independently of the height of the vacuum, therefore, a constantly continuous passage of the band through the apparatus is given. The sealing-liquid baths may at the same time serve as treatment baths, for instance in such a manner that the liquid seal at the band-admission end of the apparatus constitutes at the same time the last cleaning stage of a preparatory treatment of the band, whilst by the liquid seal at the band exit end an after-treatment of the finished band may at the same time take place, for instance in such a manner that the coated band is here coated with a thin protective film, in order to prevent an electrostatic charging, and therefore an attraction of dust.

These and further details of the process according to the invention, as well as of the apparatus according to the invention, are further explained by reference to a constructional example, which is illustrated in the accompanying drawings, in which:

FIGURE 1 shows in front elevation the apparatus according to the invention;

FIGURE 2 is a diagrammatic representation of a coating appliance known in itself;

FIGURE 3 shows a section on the line III—III in FIGURE 1; and

FIGURE 4 a section on the line IV—IV in FIGURE 3. The apparatus illustrated consists essentially of four vessels 1, 2, 3, 4, erected side by side in one plane, a vacuum tank 5 arranged above them at a higher level, and six vertically extending connecting tubes 6, 7, 8, 9, 10, 11, by which the lower vessels 1, 2, 3, 4 are connected with the vacuum tank 5. In order to ensure a satisfactory sealing, that is, a vacuum-tight sealing, of the connecting tubes 6, 7, 8, 9, 10, 11, each of the lower vessels 1, 2, 3, 4, is equipped with two upwardly directed tubular members or sockets 1a, 1b, 2a, 2b, 3a, 3b, 4a and 4b, whilst the vacuum tank 5 above them has six downwardly directed sockets, c, d, e, f, g and h. The connection of the lower vessels 1, 2, 3, and 4 with the upper vacuum tank 5 is here established by means of the connecting tubes 6, 7, 8, 9, 10 and 11 in such a way that the band 12 to be coated can be passed through the apparatus in a succession of vertical loops by way of lower reversing rollers 13, 14, 15, 16 arranged inside the vessels 1, 2, 3 and 4, and by way of upper reversing rollers 17, 18, 19 journaled in the vacuum tank 5. The open socket 1a of the vessel 1 here serves as an entry into the

apparatus, and the socket  $4a$  of the vessel  $4$  as an exit from the apparatus. The band admission roller  $20$ , and the band outlet roller  $21$ , are located at about the same level outside the apparatus itself.

All parts of the apparatus, that is, the lower vessels, the vacuum tank and the connecting tubes, may fundamentally be made of any desired cross section, even square or rectangular. A round or at least oval cross-sectional form is however preferred. The production of the vacuum is effected by vacuum-producers not represented in the drawings, such for instance as pumps, steam-jet ejectors, condensers or the like, which are connected to the upper vacuum tank  $5$  by way of tank unions  $22$ .

The vessels  $1$  and  $4$  both serve as liquid-containers for the accommodation of sealing liquid, and thus are at the same time slitudes for the air-free admission and exit of the band. The sealing medium is in both cases an aqueous solution. The solution in the vessel  $1$ , that is, at the end at which the band enters, may also pertain to the last cleaning stage of the preparatory treatment of the band. The solution in the vessel  $4$ , on the other hand, may be a special solution, which, as the coated band runs through, deposits upon the surface of the band a protective film, by which an electrostatic charging, and therefore an attraction of dust, is prevented.

During the operation, in dependence upon the height of the vacuum in the apparatus, the solutions in the vessels  $1$  and  $4$  are drawn upwards by suction into the vacuum space, that is, into the connecting tubes  $6$  and  $11$ . In each of these connecting tubes  $6$  and  $11$  a column of liquid corresponding to the vacuum accordingly adjusts itself. On the vessels  $1$  and  $4$  are also provided overflow spouts  $23$  and  $24$ , by which the solutions in these vessels flow away into a collecting receptacle located lower down and not represented in the drawing, to be pumped back again from there into the vessels by way of the sockets or pipe couplings  $1a$  and  $4a$ , which are open to the atmosphere. This has the advantage that the surface level of liquid in the vessels  $1$  and  $4$  always maintains a constant height, even if accidental fluctuations should occur in the vacuum. Furthermore in this way the composition of the solution can be constantly checked, and can be supplemented or renewed in case of need.

The vessels  $2$  and  $3$  serve as treatment vessels, and are subject to vacuum. They contain, besides the lower band-reversing rollers  $14$  and  $15$  respectively, the actual coating devices  $26$  and  $28$  respectively, for applying an adhesion-promoting medium and the layer of synthetic material respectively. Similar coating devices  $25$  and  $27$  are moreover provided in the vacuum tank  $5$ , the coating device  $25$  being designed for applying an adhesion-promoting medium and the coating device  $27$  for applying the layer of synthetic material. The adhesion promoting medium may be the proprietary preparation known as "mesamol," or some similar primer.

Each coating device, as shown in FIGURE 2, consists of a trough  $40$  containing the liquid synthetic material or the adhesion-promoting means, a dipping roller  $41$  dipping into the trough, and an applying roller  $42$  co-operating with the dipping roller. The entire unit, including its drive, is supported in the vacuum space, and each such unit is arranged in the neighbourhood of one of the reversing rollers  $14$ ,  $15$ ,  $17$  or  $18$  that guide the band  $12$ , so that during the application of the layer of synthetic material the reversing roller serves as a counter-pressure roller.

In order to enable the thickness of the coating to be accurately adjusted while it is being applied, the entire coating device is displaceable towards the band, that is, towards the centre of the reversing roller. The troughs  $40$  containing the liquid synthetic material have each an overflow connection as well as an inlet connection. These connections are in communication with a storage vessel, which is arranged outside and underneath the vacuum

plant. In order that the coating materials may not dry up, and that their viscosity may be maintained, they are continuously pumped round. For the maintenance of the vacuum it is however requisite that the connecting pipes should form a U-shaped loop extending vertically downwards and corresponding to the height of the vacuum, so as to counteract the suction produced by the vacuum.

The bottoms of the treatment vessels  $2$  and  $3$  are so constructed that in a method of working with a rather coarse vacuum of for instance more than 100 Torr, the solvent condensing on and running down the cooler walls of the tubes  $7$ ,  $8$ ,  $9$  and  $10$  can be caught underneath. By special discharge pipes  $29$  and  $30$  the condensate is drawn off, and the surface level of the condensate in the vessels  $2$  and  $3$  is maintained constant. The discharge pipes  $29$  and  $30$ , like the connecting tubes of the coating devices, are of U-shaped construction and extend vertically downwards, the length of the U-shaped loop having to be adapted to the height of the vacuum. For the satisfactory condensation of the vapourised solvent, cooling devices, for instance cooling coils  $31$ , may if desired be provided in the treatment vessels  $2$  and  $3$ . An external cooling of the vessels  $2$  and  $3$ , or of the connecting tubes  $7$ ,  $8$ ,  $9$  and  $10$ , is however likewise possible.

The treatment or coating of the band  $12$  is effected in the treatment vessels  $2$  and  $3$  and in the vacuum tank  $5$ . The connecting tubes  $6$  and  $11$  serve as drying spaces for the drying and hardening of the coating material, so that the length of the drying tract is determined by the length of the connecting tubes. By increasing the length of the connecting tubes, therefore, the length of the drying tract can be increased in a very cheap and simple manner, without the other structural parts of the apparatus having to be altered. The connecting tubes  $6$  and  $11$  communicating with the liquid vessels  $1$  and  $4$  serve at the same time as stand-pipes for the columns of sealing liquid sucked upwards by the vacuum.

In order to accelerate the drying and hardening or polymerisation of the freshly applied coating, and at the same time to make good the heat removed by vaporisation of the solvents, heating devices  $32$  are installed in the connecting tubes. Since the transfer of heat in the vacuum can only be effected by radiation, the heating devices  $32$  are preferably infra-red radiators or similar thermal radiators. These heating devices are located near the band surface just coated, and are so arranged that an intensive irradiating of the coating substances is possible.

One form of construction, by way of example, of a heating appliance constructed as a thermal radiator, is shown by FIGURES 3 and 4. The thermal radiator elements are assembled into groups, each group of radiators consisting of a number of tubes  $34$  arranged transversely to the direction in which the band passes, and welded in a vacuum-tight manner to the connecting tube, for instance to the tube  $7$  in FIGURES 3 and 4. The thermal radiating tubes  $34$  are open at both ends, so that any desired source of heat can be fitted in or connected thereto. For the strengthening and intensifying of the radiating effect, reflectors  $35$  are provided on the side of the thermal radiating tubes  $34$  remote from the band  $12$ , as shown in FIGURE 4.

If the connecting tubes  $7$  to  $10$  are provided throughout their length with such radiating tubes  $34$ , they admit of being used optionally for heating or for cooling. In this way the entire apparatus can be widely adapted to all coating requirements.

The working procedure or coating operation in the apparatus according to the invention is as follows: The band  $12$  to be coated is introduced, by way of the band-entry roller  $20$ , through the open tubular member  $1a$ , into the liquid vessel  $1$ , and is guided upwards by the reversing roller  $13$ , journaled in the liquid, into the connecting tube  $6$ . In the upper part of the connecting tube  $6$  is mounted a heating device  $32$ , which vaporises drops of water that

have remained clinging by adhesion to the surface of the band. Upon the deflection of the band 12 round the upper reversing roller 17, an adhesion-promoting medium is applied to one side of the band by the coating device 25. Upon the further travel of the band this applied layer is irradiated by the heating device 32 located in the connecting tube 7, the solvent evaporating and the coating itself being dried out. In the treatment vessel 2, by means of the coating device 26, the other side of the band is then provided with an adhesion-promoting medium, which, upon the band ascending again, is dried in the connecting tube 8. As the band passes round the upper deflecting roller 18, the first side of the band is now coated with a synthetic material, which, during the further travel through the connecting tube 9, is hardened or polymerised by the aid of the heating device 32 therein. Then in the treatment vessel 3 the coating of the second side of the band with synthetic material is effected as it passes round the deflecting roller 15, the hardening or polymerisation being effected in the succeeding connecting tube 10. By the upper deflecting roller 19 the band 12 is deflected downwards again, and dips, in the connecting tube 11, into the liquid seal of the liquid-container 4. After deflection of the band by the lower reversing roller 16, journaled in the liquid container 4, the band then leaves the apparatus through the open tubular member 4a to be guided away over the band exit roller 21.

Immediately before the coating appliances 27, 28 that apply the coating of synthetic material, further heat-radiating devices may be provided, for the purpose of transiently softening by heat the adhesion-promoting coating already applied. A better adhesion of the layer of synthetic material can be obtained in this way, according to the consistency of the coating substances.

I claim:

1. Apparatus for applying thin synthetic coatings to metal bands and hardening the coatings, comprising: a closed liquid container formed with an inlet for the band to be coated, a closed liquid container formed with an outlet for the coated band, treatment vessels located between the two liquid containers and at the same level, a vacuum tank located above the liquid containers and treatment vessels, a connecting tube extending upwards from each liquid container to the vacuum tank, two connecting tubes extending upwards from each treatment vessel to the vacuum tank, reversing rollers so arranged in the liquid containers, treatment vessels and vacuum tank that a band entering the first liquid container through the band inlet can pass round the reversing rollers and through the liquid containers, treatment vessels, vacuum tank and connecting tubes in a plurality of vertical loops to the band outlet, means for exhausting air from the vacuum tank,

the treatment vessels and the tubes connecting them with one another, means in the treatment vessels for applying a solution of synthetic coating material in an at least semi-liquid condition to that side of the band that does not come into contact with the rollers therein, means in the vacuum tank for applying synthetic coating material in an at semi-liquid condition to that side of the band that does not come into contact with the reversing rollers in the vacuum tank, and means in the connecting tubes for heating that side of the band which in each case had not come into contact with the preceding reversing roller.

2. Apparatus for applying thin synthetic coatings to metal bands and hardening the coatings as claimed in claim 1, the heating means in the connecting tubes being infra-red radiators.

3. Apparatus for applying thin synthetic coatings to metal bands and hardening the coatings as claimed in claim 1, further comprising: cooling means for condensing the vapours of the solvent removed from the synthetic coating by the heating means, and discharged pipes for removing excess condensed solvent from the treatment vessels without disturbing the vacuum therein.

4. A method for the bubble-free application of thin coatings of synthetic material, in a continuous operation, to a continuously advancing metal band, and for the rapid hardening of the coatings applied, comprising: bringing the synthetic material into an at least semi-liquid condition by means of a solvent, applying this semi-liquid material to the band in a partial vacuum, hardening or polymerizing the coating so applied, still in a partial vacuum, the height of the vacuum being such that the vaporization temperature of the solvent is at about room temperature, and replacing the heat of vaporization, which is withdrawn from the synthetic material in the vaporization of the solvent, by thermal radiation from an external source.

#### References Cited by the Examiner

##### UNITED STATES PATENTS

|    |           |         |          |       |           |
|----|-----------|---------|----------|-------|-----------|
| 40 | 987,629   | 3/1911  | Ketchson | ----- | 117—61 X  |
|    | 1,069,033 | 7/1913  | Rowland  | ----- | 118—61    |
|    | 1,322,327 | 11/1919 | Minton   |       |           |
|    | 1,331,729 | 2/1920  | Taylor   | ----- | 117—61    |
|    | 1,595,236 | 8/1926  | Minton   | ----- | 117—61    |
| 45 | 1,595,475 | 8/1926  | Minton   | ----- | 117—61    |
|    | 2,137,256 | 11/1938 | Waldron  | ----- | 117—61 X  |
|    | 2,346,523 | 4/1944  | Vincent  | ----- | 117—61    |
|    | 2,894,483 | 7/1959  | Stahl    | ----- | 118—50    |
| 50 | 2,937,108 | 5/1960  | Toye     | ----- | 117—119 X |

MURRAY KATZ, Primary Examiner.

JOSEPH B. SPENCER, Examiner.